

## 1

2,793,131

**THERMAL INSULATING SHAPE AND METHOD OF MANUFACTURE**

Mark E. Binkley, Somerville, N. J., assignor to Johns-Manville Corporation, New York, N. Y., a corporation of New York

No Drawing. Application May 3, 1952,  
Serial No. 286,010

14 Claims. (Cl. 106—121)

This invention relates to insulating blocks or shapes and more particularly to high temperature insulating shapes incorporating silica in the form of diatomaceous earth as a major ingredient.

The high temperature insulation shape and method of manufacture which form the subject of the present invention represent improvements on the High Temperature Insulating Shapes and Methods of Manufacture which are described in United States Patent No. 2,033,106 granted March 3, 1936 to Arthur B. Cummins and Patent No. 2,388,549 granted November 6, 1945 to Henry A. Kieselbach and Earl R. Williams.

Insulating blocks of the type described in the Cummins patent develop considerable shrinkage during the period of manufacture and cannot, therefore, be molded to precise dimensions. Such blocks must be molded and thereafter planed down or trimmed to the desired dimensions for their intended use. The manufacture of finished blocks by such a method is, therefore, costly and time consuming and involves considerable loss of material in the form of trimming waste. The insulating blocks and method of their manufacture disclosed in the Kieselbach and Williams patent are an improvement upon those defined in the Cummins patent in that the composition of the blocks therein disclosed is such as to eliminate a substantial proportion of the shrinkage of such insulating bodies and to enable molding of the bodies to relatively true dimensions.

Various disadvantages, however, have been found in the block and method of manufacturing the same, as disclosed in the Kieselbach and Williams patent. Probably the primary disadvantage is the inability to employ the disclosed composition and procedure to fabricate insulating bodies for use at high temperatures, such as 2000° F., having a desirable low density as, for example, a density of approximately 20 lbs./cu. ft. If such light weight products are formed in accordance with the Kieselbach and Williams procedure, they are generally unstable in insulating service at temperatures ranging in the neighborhood of 2000° F., due to the necessity of using a relatively high percentage of magnesium carbonate in the block to obtain such densities. While such blocks do not have the serious shrinkage characteristics of those defined in the Cummins patent, they still do exhibit shrinkage in an undesirable amount. Furthermore, the procedure outlined in the Kieselbach and Williams patent entails the step of casting the material or utilizing a plate and frame type filter press to form the body. Either manufacturing procedure, therefore, requires the provision of a large number of molds during forming and curing, thereby rendering the procedure relatively slow and expensive.

Accordingly, it is an object of the present invention to provide an improved method of manufacturing insulating shapes, particularly high temperature insulating shapes incorporating diatomaceous silica as a principal ingredient, whereby such shapes can be molded and cured to precise dimensions.

## 2

A more particular object of the present invention is to provide a precision piston press filter molded heat insulation shape adapted for use at elevated temperatures in the neighborhood of 2000° F. and having improved strength and insulation capacity during low or high temperature insulation service.

A further object of the present invention is to provide a filter molded insulating shape adapted for use in high temperature insulating service and having a substantially lower density than heretofore obtained with insulating materials of comparable composition.

With the above and other objects and features in view, the invention consists in the improved insulating shapes and a method of manufacture hereinafter described and more particularly defined in the appended claims.

The insulation shape which forms the subject of the present invention incorporates diatomaceous earth as a principal ingredient. The composition of the herein-described insulating bodies is somewhat similar to that defined in the Kieselbach and Williams patent and particularly differs from that disclosed in the Cummins patent in the same manner as does the patent to Kieselbach and Williams; that is, the composition herein-described differs from the Cummins patent in that the principal bonding agent which is used in the manufacture of bodies in accordance with the invention comprises self-setting normal magnesium carbonate, rather than preformed basic magnesium carbonate. The composition of the blocks formed in accordance with this invention primarily differs from that defined in the Kieselbach and Williams patent in the inclusion of a relatively small amount of lime in the modifiable slurry composition containing diatomaceous silica, staple reinforcing fibers, and normal magnesium carbonate crystals.

35 Suitable blocks formed in accordance with this invention are molded from a relatively dilute slurry essentially containing, in percent of solids by weight, approximately 35-78% of diatomaceous earth, approximately 5-15% of staple reinforcing fiber, preferably asbestos fiber, approximately 2-7% of lime, preferably hydrated lime, approximately 0-10% bentonite clay, and approximately 5-50% of self-setting normal magnesium carbonate in the form commonly referred to as "A" crystals of magnesium carbonate. The preferred blocks of this invention are suitable for high temperature insulating service as, for example, in the neighborhood of 2000° F. and preferably comprise the heat reaction product of a wet molded mixture containing, in percent of solids by weight, approximately 60-75% of calcined diatomaceous earth particles, approximately 10-12% of asbestos fiber, approximately 4-6% of lime, preferably hydrated, approximately 5-7% of bentonite clay, and approximately 14-22% of self-setting normal magnesium carbonate crystals.

55 As may be clearly seen, the slurry composition used in this invention to form suitable insulating shapes contains a relatively small but significant amount of lime. Heretofore, lime has been purposely excluded from blocks of compositions comparable to those utilized in accordance with this invention since the presence in the slurry of even a small amount of lime causes deterioration of the magnesium carbonate required for the binder matrix. The incorporation of the lime in the molding slurry, and hence in the finally fabricated insulating body, in accordance with this invention, does not detrimentally affect the block; conversely, its use has been found to result in an insulating shape which exhibits, as compared to conventional insulating shapes of comparable compositions and those defined in the Cummins and Kieselbach and Williams patents, no substantial shrinkage from the wet precision molded form to that of the finally cured and dried body, ready for insulating service.

The procedure of manufacture utilized to form the insulating bodies of this invention essentially comprises forming voluminous flocks of lightly bonded, interlaced, self-setting normal magnesium carbonate crystals and staple reinforcing fibers in dilute aqueous suspension; mixing with the aqueous slurry of such flocks a substantial amount of a gelled slurry of diatomaceous earth, lime, staple reinforcing fiber, and, preferably, bentonite; partially dewatering and molding the wet solids content of the mixed slurry under pressure; immediately removing the formed body from the mold; and developing a shape-retaining set of the thus formed body by heating.

As an initial step in the process, an aqueous slurry of voluminous flocks of lightly bonded, interlaced, self-setting normal magnesium carbonate crystals and staple reinforcing fibers is formed. Preferably, normal magnesium carbonate crystals are obtained by precipitating normal magnesium carbonate from a magnesium bicarbonate solution by subjecting the bicarbonate solution to severe agitation, as by aeration, at a temperature within the range 100-120° F. After most of the magnesium bicarbonate has been converted to normal carbonate, the slurry is cooled to a temperature about 80° F. to stabilize the normal magnesium carbonate. The slurry is then concentrated to a solids content preferably exceeding 15% by weight, as by filtering or by decantation.

By limiting the time of aerating a solution of magnesium bicarbonate liquor of, say, 3% concentration (basic magnesium carbonate equivalent) within a period of about one hour at a temperature of 80-130° F. with thorough agitation, as in a turbo-aerator, a reactive form of elongated orthorhombic normal magnesium carbonate crystals can be produced having an average dimension of 20-40 microns in length and 2-4 microns in maximum thickness.

A portion of the staple reinforcing fibers to be used in the insulating body of this invention is then added to the total required amount of normal magnesium carbonate crystal slurry in proportions normally ranging between 8 and 25% by weight of the normal magnesium carbonate crystals, or approximately 0.4-12.5% by weight of the solids in the finally formed molding slurry. The temperature of the thus formed fiber-crystal slurry should not at any time exceed about 120° F. up to this point. The relatively cool fiber-crystal slurry is then diluted with a measured volume of hot water at a temperature above 140° F. and preferably between 180 and 210° F. The concentration of slurry solids after such dilution should preferably range from 1-8.5% by weight. The thus mixed hot water and slurry are agitated to secure a uniform suspension of slurry solids, after which the dilute slurry charge is allowed to stand quiescent until large flocks of crystal-fiber aggregates of substantial water-retaining capacity, somewhat resembling in appearance thick, incompletely cooked oatmeal porridge, are formed.

The temperature of the charge during the period of quiescent standing should be above 140° F., and the upper temperature is limited by the temperature of the diluting water and will not exceed 210° F. Usually the slurry temperature will range between 140 and 180° F., and preferably within the range 150-170° F. The length of the period of quiescent standing to develop flocculation depends primarily upon the temperature of the slurry and should preferably range between 2 and 32 minutes. For example, when it takes eight minutes for a slurry of predetermined solids concentration to develop a flocculent or oatmeal condition at a temperature of 160° F., it has been found that a period of about four minutes quiescent standing is necessary for a slurry of the same concentration to react to a flocculent state at a temperature of 170° F. As is apparent, the time of quiescent standing decreases as the prereaction temperature of the slurry increases.

The thus formed bonded, interlaced fiber-crystal flocks have sufficient cohesive strength so that they do not settle appreciably while in dilute aqueous suspension and have exceptionally high water-retaining capacity, which characteristics contribute to the light density of the blocks formed in accordance with this invention.

While this "oatmeal" slurry is being produced, a separate slurry is formed with the diatomaceous earth, lime, the remainder of the staple reinforcing fiber, and bentonite, if used. Preferably, these ingredients are initially added to sufficient water to form a mixture having approximately the consistency of a thick mud. This initial mixing operation is followed by a treatment designed to develop extensive prereaction, flocculation, and volume expansion of the solids to improve the water-retaining capacity and gel characteristics of the mixture. As a preliminary to this prereaction operation, this mixture is diluted with water to form a slurry preferably containing at least about eight parts by weight of water to one part of solids. Within such a dilute slurry it is possible to obtain optimum volume expansion and formation of a prereacted lime and silica gel having good bulking, water-retaining, and free filtering characteristics desirable for the formation of the blocks of this invention. If bentonite is used in the composition, as is preferred for light weight, high temperature, insulating blocks, the lime also serves to flocculate the bentonite, which in turn adds additional gel structure to the slurry and gives it better bulking, water-retaining, and free filtering characteristics.

This prereaction gel-forming treatment is carried out by quiescent reaction in the slurry at an elevated temperature in the range of approximately 170-210° F. for at least forty-five minutes. Preferably, the slurry is heated to a temperature of approximately 190-205° F. and allowed to stand quiescent with periodic mild agitation for the desired period of time. Additional standing time is not detrimental to the formation of the insulating blocks fabricated in accordance with this invention since the bonding matrix of the blocks is not dependent upon the formation of a calcium silicate.

After both the "oatmeal" slurry and the gel have been formed, they are mixed together to well disperse the flocks of each slurry, and the mixed slurry is then charged to a mold. As hereinbefore indicated, the mixed slurry thus formed is particularly adapted for piston press filter molding of the blocks of this invention. While it is clear that the slurry may be molded by conventional slower methods, such as in a plate and frame type filter press, it is apparent that piston press filter molding is ideal to enable the rapid formation of light weight insulating bodies with the use of a minimum of apparatus. When the pre-reacted mixed slurry is transferred into the piston press, drainage of water starts immediately and is accelerated by the descent of the piston toward the mold base screen. As the piston descends within the mold, the solids content of a mold charge is compressed to precise final block dimensions under mechanical pressures, which, during at least the initial stages of the molding operation, should be as high as 60 lbs./sq. in. when molding blocks of, for example, 20 lbs./cu. ft. density.

The wet molded-block as made in accordance with the present invention has adequate compressible strength so that it may be immediately removed from the supporting mold base for transfer to a drying oven preferably operated at a temperature of approximately 220-350° F., wherein the normal magnesium carbonate in the body is converted to basic magnesium carbonate to form the binder matrix thereof.

As a specific example of this invention a high temperature insulating block was formed in the following manner: Into 15 gallons of water were mixed 1.0 lb. of amosite asbestos fibers, 0.6 lb. bentonite-clay, 6.4 lbs. of finely divided calcined diatomaceous earth, and 0.5 lb. of hydrated lime. The thus formed slurry was heated to

200° F. and then allowed to stand quiescent for one hour, during which time the slurry solids gelled with flocculation and substantial volume expansion. Similarly, 1.2 gal. of a slurry containing 2.5 lbs. of self-setting normal magnesium carbonate "A" crystals and 0.25 lb. of amosite asbestos fiber was diluted with 5 gals. of water which had a temperature of 195° F. This diluted slurry was mixed by air or mechanical agitation for approximately 2 minutes and allowed to stand quiescent for about 10 minutes, during which time large flocks of crystal-fiber aggregates of substantial water-retaining capacity formed. The gelled slurry containing the diatomaceous earth was then mixed with the thus formed fiber-crystal "oatmeal" slurry, and the mixed slurry charged to a filtering piston press wherein the block was precisely molded to dimensions of 2" in thickness, 12" in width, and 36" in length. After molding, the block was immediately removed from the mold and dried for 48 hours at 300° F., without exhibiting dimensional change. The thus formed block had a density of 20 lbs./cu. ft. and a modulus of rupture of 64 lbs./sq. in. and easily withstood the soaking heat at insulating service temperatures of 2000° F.

When utilizing the hereinbefore disclosed procedure and slurry compositions, the insulating shapes of this invention may be molded to precise dimensions and exhibit no substantial amount of shrinkage in volume during the molding, curing, and drying operations. The high temperature insulating blocks according to the hereinbefore-defined preferred composition exhibit this non-shrinking characteristic during molding and drying, and also exhibit an excellent resistance to shrinkage at insulating service temperatures of approximately 2000° F. For example, a high temperature block of the preferred composition of this invention shrinks less than 2% linearly as compared to over 3% for those formed in accordance with the Kieselbach and Williams procedure. Additionally, these high temperature insulating blocks are not destroyed by soaking heat at these high temperatures, as are conventional magnesia insulating bodies. The blocks according to this invention have substantially dust-free, hard surfaces containing filter screen impressions and have a lower density and a higher ratio of modulus of rupture to density than comparable insulating blocks heretofore fabricated without using normal magnesium carbonate crystals. Blocks made in accordance with the present invention have a modulus of rupture to density ratio of at least 3 throughout the preferred density range of 15-25 lbs./cu. ft. and have a substantially lesser density for the same composition when compared to the insulating bodies formed in accordance with the hereinbefore-mentioned Kieselbach and Williams patent.

Preferably, the diatomaceous earth utilized in the blocks should be reduced to finely divided or powdered form and, for blocks formed for high temperature insulating service, should be straight or flux calcined at temperatures not substantially less than the insulating service temperature at which the block will be used. In similar manner, the lime and bentonite utilized in this block should be in finely divided form to enable the formation of the desired gelled slurry. Asbestos fiber, preferably amosite fiber, is the most suitable staple reinforcing fiber for use in this invention, but conventional reinforcing fibers such as mineral wool, glass, etc., may be utilized to provide the bulking structure for the gelled and "oatmeal" slurries.

It will be understood that the details given are for the purpose of illustration, not restriction, and that variations within the spirit of the invention are intended to be included in the scope of the appended claims wherein the percentages set forth are in percent by weight of solids in the finally formed and molded slurry unless otherwise indicated.

What I claim is:

1. The method of manufacturing light weight insulat-

ing shapes which comprises forming an aqueous slurry containing approximately 5-50% self-setting normal magnesium carbonate crystals and approximately 0.4-12.5% staple reinforcing fibers having a temperature below approximately 120° F., rapidly diluting and heating said slurry with hot water at a temperature and in amount sufficient to raise the temperature of the slurry to approximately 140-210° F., maintaining the thus diluted and heated slurry quiescent for 2-32 minutes to develop therein voluminous flocks of lightly bonded interlaced crystals and fiber, mixing with said fiber-crystal slurry a gelled aqueous slurry formed by subjecting a slurry containing approximately 35-78% diatomaceous earth, approximately 2-7% lime and approximately 2.5-14.6% staple reinforcing fiber and having a water to solids ratio of at least 8 to 1 to quiescent reaction of said lime and diatomaceous earth at a temperature of approximately 170-210° F. for at least 45 minutes, partially dewatering and molding the wet solids content of the thus mixed slurry under pressure, and developing a shape-retaining set of the molded shape by heat to convert the normal magnesium carbonate crystals to magnesium basic carbonate.

2. The method of manufacturing light weight insulating shapes which comprises forming an aqueous slurry containing approximately 5-50% self-setting normal magnesium carbonate crystals and approximately 0.4-12.5% staple reinforcing fibers having a temperature below approximately 120° F., rapidly diluting and heating said slurry with hot water at a temperature and in amount sufficient to raise the temperature of the slurry to approximately 140-210° F., maintaining the thus diluted and heated slurry quiescent for 2-32 minutes to develop therein voluminous flocks of lightly bonded interlaced crystals and fiber, mixing with said fiber-crystal slurry a gelled aqueous slurry formed by subjecting a slurry containing approximately 35-78% diatomaceous earth, approximately 2-7% lime, up to 10% bentonite and approximately 2.5-14.6% staple reinforcing fiber and having a water to solids ratio of at least 8 to 1 to quiescent reaction of said lime and diatomaceous earth at a temperature of approximately 170-210° F. for at least 45 minutes, partially rewetting and molding the wet solids content of the thus mixed slurry under pressure, and developing a shape-retaining set of the molded shape by heat to convert the normal magnesium carbonate crystals to magnesium basic carbonate.

3. The method of manufacturing light weight high temperature insulating shapes which comprises forming an aqueous slurry containing approximately 14-22% self-setting normal magnesium carbonate crystals and approximately 1-5.5% staple reinforcing fibers having a temperature below approximately 120° F., rapidly diluting and heating said slurry with hot water at a temperature and in amount sufficient to raise the temperature of the slurry to approximately 140-210° F., maintaining the thus diluted and heated slurry quiescent for 2-32 minutes to develop therein voluminous flocks of lightly bonded interlaced crystals and fiber, mixing with said fiber-crystal slurry a gelled aqueous slurry formed by subjecting a slurry containing approximately 60-75% diatomaceous earth, approximately 4-6% lime and approximately 4.5-11% staple reinforcing fiber and having a water to solids ratio of at least 8 to 1 to quiescent reaction of said lime and diatomaceous earth at a temperature of approximately 170-210° F. for at least 45 minutes, partially dewatering and molding the wet solids content of the thus mixed slurry under pressure, and developing a shape-retaining set of the molded shape by heat to convert the normal magnesium carbonate crystals to magnesium basic carbonate.

4. The method of manufacturing light weight high temperature insulating shapes which comprises forming an aqueous slurry containing approximately 14-22% self-setting normal magnesium carbonate crystals and approxi-

mately 1-5.5% staple reinforcing fibers having a temperature below approximately 120° F., rapidly diluting and heating said slurry with hot water at a temperature and in amount sufficient to raise the temperature of the slurry to approximately 140-210° F., maintaining the thus diluted and heated slurry quiescent for 2-32 minutes to develop therein voluminous flocks of lightly bonded interlaced crystals and fiber, mixing with said fiber-crystal slurry a gelled aqueous slurry formed by subjecting a slurry containing approximately 60-75% diatomaceous earth, approximately 4-6% lime, approximately 5-7% bentonite and approximately 4.5-11% staple reinforcing fiber and having a water to solids ratio of at least 8 to 1 to quiescent reaction of said lime and diatomaceous earth at a temperature of approximately 170-210° F. for at least 45 minutes, partially dewatering and molding the wet solids content of the thus mixed slurry under pressure, and developing a shape-retaining set of the molded shape by heat to convert the normal magnesium carbonate crystals to magnesium basic carbonate.

5. A precision molded, light weight thermal insulating body comprising the heat reaction product of a wet molded mixture of approximately 5-50% self-setting normal magnesium carbonate crystals, approximately 35-78% finely divided diatomaceous earth, approximately 2-7% lime, and approximately 5-15% staple reinforcing fiber, said lime being present in the form of a hydrous calcium silicate from reaction with diatomaceous earth.

6. A precision molded, light weight thermal insulating body comprising the heat reaction product of a wet molded mixture of approximately 5-50% self-setting normal magnesium carbonate crystals, approximately 35-78% finely divided diatomaceous earth, approximately 2-7% lime, up to 10% bentonite, and approximately 5-15% staple reinforcing fiber, said lime being present in the form of a hydrous calcium silicate from reaction with diatomaceous earth.

7. A precision filter molded thermal insulating body having a density of approximately 15-25 lbs./cu. ft. and a modulus of rupture to density ratio of at least 3, comprising the heat reaction product of a wet molded mixture of approximately 5-50% self-setting normal magnesium carbonate crystals, approximately 35-78% finely divided diatomaceous earth, approximately 2-7% lime, and approximately 5-15% staple reinforcing fiber, said lime being present in the form of a hydrous calcium silicate from reaction with diatomaceous earth.

8. A precision molded thermal insulating body having a density of approximately 15-25 lbs./cu. ft. and a modulus of rupture to density ratio of at least 3, comprising the heat reaction product of a wet molded mixture of approximately 5-50% self-setting normal magnesium carbonate crystals, approximately 35-78% finely divided diatomaceous earth, approximately 2-7% lime, up to 10% bentonite, and approximately 5-15% staple reinforcing fiber, said lime being present in the form of a hydrous calcium silicate from reaction with diatomaceous earth.

9. A precision molded thermal insulating body adapted for use in high temperature insulating service, comprising the heat reaction product of a wet molded mixture of approximately 14-22% self-setting normal magnesium carbonate crystals, approximately 60-75% finely divided diatomaceous earth, approximately 4-6% lime, approximately 5-7% bentonite, and approximately 10-12% asbestos fiber, said lime being present in the form of a hydrous calcium silicate from reaction with diatomaceous earth.

10. A precision molded thermal insulating body adapted for use in high temperature insulating service and having a density of approximately 15-25 lbs./cu. ft. and a modulus of rupture to density ratio of at least 3, comprising the heat reaction product of a wet molded mixture of approximately 14-22% self-setting normal magnesium carbonate crystals, approximately 60-75%

finely divided diatomaceous earth, approximately 4-6% lime, approximately 5-7% bentonite, and approximately 10-12% asbestos fiber, said lime being present in the form of a hydrous calcium silicate from reaction with diatomaceous earth.

11. The method of manufacturing light weight insulating shapes which comprises forming an aqueous slurry of lightly bonded voluminous flocks of approximately 5 to 50% self-setting normal magnesium carbonate crystals and approximately 0.4 to 12.5% staple reinforcing fiber, said lightly bonded voluminous flocks being formed by maintaining a dilute slurry of the normal magnesium carbonate crystals and staple reinforcing fiber at a temperature of approximately 140 to 210° F. for a period of about 2 to 32 minutes, mixing with said fiber-crystal slurry a gelled aqueous slurry containing approximately 35 to 78% diatomaceous earth, approximately 2 to 7% lime and approximately 2.5 to 14.6% of staple reinforcing fiber, said gelled aqueous slurry being formed by maintaining a dilute slurry of the diatomaceous earth, lime and staple reinforcing fiber at a temperature of approximately 170 to 210° F. for at least 45 minutes, partially dewatering the wet solids content of the thus formed mixed slurry, and developing a shape-retaining set of the molded shape by heating to convert the normal magnesium carbonate crystals to magnesium basic carbonate.

12. The method of manufacturing light weight insulating shapes which comprises forming an aqueous slurry of lightly bonded voluminous flocks of approximately 5 to 50% self-setting normal magnesium carbonate crystals and approximately 0.4 to 12.5% staple reinforcing fiber, said lightly bonded voluminous flocks being formed by maintaining a dilute slurry of the normal magnesium carbonate crystals and staple reinforcing fiber at a temperature of approximately 140 to 210° F. for a period of about 2 to 32 minutes, mixing with said fiber-crystal slurry a gelled aqueous slurry containing approximately 35 to 78% diatomaceous earth, approximately 2 to 7% lime, up to 10% bentonite and approximately 2.5 to 14.6% staple reinforcing fiber, said gelled aqueous slurry being formed by maintaining a dilute slurry of the diatomaceous earth, lime, bentonite and staple reinforcing fiber at a temperature of approximately 170 to 210° F. for at least 45 minutes, partially dewatering and molding the wet solids content of the thus formed mixed slurry, and developing a shape-retaining set of the molded shape by heating to convert the normal magnesium carbonate crystals to magnesium basic carbonate.

13. The method of manufacturing light weight insulating shapes which comprises forming an aqueous slurry containing, in percent of solids by weight, approximately 5 to 50% self-setting normal magnesium carbonate crystals and approximately 0.4 to 12.5% staple reinforcing fiber, heating said slurry to raise its temperature to approximately 140 to 210° F., maintaining the thus heated slurry quiescent for about 2 to 32 minutes to develop therein voluminous flocks of lightly bonded interlaced crystals and fiber, mixing with said fiber-crystal slurry a gelled aqueous slurry formed by subjecting a slurry containing, in percent of solids by weight, approximately 35 to 78% diatomaceous earth, approximately 2 to 7% lime and approximately 2.5 to 14.6% staple reinforcing fiber and having a water to solids ratio of at least 8 to 1 to quiescent reaction of said lime and diatomaceous earth at a temperature of approximately 170 to 210° F. for at least 45 minutes, partially dewatering and molding the wet solids content of the thus mixed slurry, and developing a shape-retaining set of the molded shape by heat to convert the normal magnesium carbonate crystals to magnesium basic carbonate.

14. The method of manufacturing light weight insulating shapes which comprises forming an aqueous slurry containing, in percent of solids by weight, approximately

5 to 50% self-setting normal magnesium carbonate crystal and approximately 0.4 to 12.5% staple reinforcing fiber, heating said slurry to raise its temperature to approximately 140 to 210° F., maintaining the thus heated slurry quiescent for about 2 to 32 minutes to develop 5 therein voluminous flocks of lightly bonded interlaced crystals and fiber, mixing with said fiber-crystal slurry a gelled aqueous slurry formed by subjecting a slurry containing, in percent of solids by weight, approximately 35 to 78% diatomaceous earth, approximately 2 to 7% lime, 10 up to 10% bentonite and approximately 2.5 to 14.6% staple reinforcing fiber and having a water to solids ratio of at least 8 to 1 to quiescent reaction of said lime and diatomaceous earth at a temperature of approximately 170 to 210° F. for at least 45 minutes, partially dewatering and molding the wet solids content of the thus mixed 15

slurry, and developing a shape-retaining set of the molded shape by heat to convert the normal magnesium carbonate crystals to magnesium basic carbonate.

References Cited in the file of this patent

UNITED STATES PATENTS

|           |                         |               |
|-----------|-------------------------|---------------|
| 1,279,975 | Boeck et al. -----      | Feb. 24, 1918 |
| 1,819,893 | Grieder -----           | Aug. 18, 1931 |
| 2,033,106 | Cummins -----           | Mar. 3, 1936  |
| 2,209,754 | Abrahams et al. -----   | July 30, 1940 |
| 2,275,032 | Greider et al. -----    | Mar. 3, 1942  |
| 2,388,549 | Kieselbach et al. ----- | Nov. 6, 1945  |
| 2,415,647 | MacArthur et al. -----  | Feb. 11, 1947 |
| 2,428,555 | Cummins et al. -----    | Oct. 7, 1947  |
| 2,536,073 | McGarvey -----          | Jan. 2, 1951  |